

W. E. HANNA.

METHOD OF HOT ROLLING EXTREMELY THIN STEEL SHEETS.  
APPLICATION FILED DEC. 6, 1920.

1,426,730.

Patented Aug. 22, 1922.



WITNESSES

J. Herk Bradley.

INVENTOR

William E. Hanna  
By Green & McCallister  
attorneys.

# UNITED STATES PATENT OFFICE.

WILLIAM E. HANNA, OF BRACKENRIDGE, PENNSYLVANIA, ASSIGNOR TO VALLEY HOLDING CORPORATION, OF BRACKENRIDGE, PENNSYLVANIA, A CORPORATION OF PENNSYLVANIA.

## METHOD OF HOT-ROLLING EXTREMELY THIN STEEL SHEETS.

1,426,730.

Specification of Letters Patent. Patented Aug. 22, 1922.

Application filed December 6, 1920. Serial No. 428,487.

To all whom it may concern:

Be it known that I, WILLIAM E. HANNA, a citizen of the United States, and a resident of Brackenridge, in the county of Allegheny and State of Pennsylvania, have made a new and useful Invention in Method of Hot-Rolling Extremely Thin Steel Sheets, of which the following is a specification.

This invention relates to the manufacture of steel sheets of extreme thinness.

In U. S. Letters Patent No. 1,340,149, issued to Vere B. Browne on May 18, 1920, there is disclosed a method of manufacturing sheets of extreme thinness, of which this method is an improvement.

In experimenting with the method disclosed in said patent, I discovered that I can materially increase the output thereunder, especially in the production of silicon steel sheets of extreme thinness.

I discovered that instead of placing relatively thin sheets of silicon steel singly between the heavier sheets or bars of dissimilar steel as outlined in said patent, I can group 25 two, three or four of such relatively thin sheets of silicon steel together between heavier sheets or bars of dissimilar steel raised to rolling temperature, and after the thin sheets are reduced to the required degree of thinness or gage, can then open up the pack.

The single sheet of drawings forming a part of this application diagrammatically illustrates a pack built up in accordance with this invention.

35 I find that all of the relatively thin sheets of such a group absorb sufficient heat for rolling and do not weld one to the other nor to the relatively heavy sheets between which the group is rolled down. The thin sheets, 40 I find, do not weld one to the other, because the temperature thereof is too low to effect welding and the outside sheets of the group do not weld to the relatively heavy sheets or bars because of the dissimilarity in the metal- 45 als; the mild steel flows more rapidly or readily than the silicon steel thus preventing welding.

The temperature absorbed by the silicon steel sheets is sufficient, since these must be 50 rolled at a low temperature on account of their silicon content. The heavy outside sheets of the pack protect the silicon steel

sheets during the rolling. I find that if I group more than four silicon steel sheets together, they have a tendency to wrinkle or 55 fold and I have found that in commercial practice, a group of four such sheets is the limit to which I can go.

In carrying out this method, I preferably take two sheets of silicon steel rolled to 29 gage (.014 of an inch), give to each of these a charcoal wash, then place or group them together between two pickled bars or relatively heavy sheets of mild or soft steel, raised to low rolling temperature, corresponding to a dark color. The pack thus made up is then rolled to from 72 to 78 inches in length, opened up and each of the silicon steel sheets is then cut into two pieces. These are given another charcoal wash and 70 new packs assembled, each of which consists of three sheets of silicon steel grouped together and inserted between other pickled bars or heavy sheets of mild or soft steel, raised to a low rolling temperature. The 75 packs are then rolled to such length as will bring the silicon steel sheets down to the desired gage or thickness, .002 or .003 of an inch as is required.

I find that the packs may be readily 80 opened and that the silicon steel sheets when thus rolled will not weld or stick one to the other, nor to the relatively heavy sheets of mild steel.

Having thus described my invention, what 85 I claim is:—

1. The method which consists in grouping two silicon steel sheets while cold, in placing such group between pickled bars of mild steel raised to rolling temperature, in rolling 90 the pack thus made up to 72 inches or more in length, in separating the pack, cutting each of the silicon steel sheets into two pieces, re-grouping two or more of these cut sheets together and inserting such group between pickled bars or relatively heavy sheets of mild steel, raised to rolling temperature and then rolling the pack to such length as will give the desired thickness to the silicon 95 steel sheets.

2. The method which consists in grouping a plurality of silicon steel sheets in a cold state between pickled bars of steel of dissimilar characteristics raised to rolling tem- 100

perature, in rolling the pack thus made up, rolling the pack to such length as will give in separating the rolled pack, cutting each silicon steel sheet into two sheets, re-grouping a plurality of these cut sheets together and between pickleled bars or relatively heavy sheets of steel of dissimilar characteristics raised to rolling temperature, and then

10  
In testimony whereof, I have hereunto subscribed my name this 2nd day of December, 1920.

WILLIAM E. HANNA.